

July 26, 1966

E. P. SADOWSKI ET AL

3,262,823

MARAGING STEEL

Filed June 7, 1963



INVENTORS  
EDWARD P. SADOWSKI  
RAYMOND F. DECKER  
BY

*W. P. Sadowski*  
ATTORNEY

## 1

3,262,823

## MARAGING STEEL

Edward P. Sadowski, Metuchen, and Raymond F. Decker, Fanwood, N.J., assignors to The International Nickel Company, Inc., New York, N.Y., a corporation of Delaware

Filed June 7, 1963, Ser. No. 286,365

12 Claims. (Cl. 148—142)

The present invention relates to high strength steel and, more particularly, to an exceedingly tough, controlled, high strength maraging steel especially usable as plate and as welded structures made from said plate.

It is well known that many steels can be used in the form of plate having a thickness from below 0.5 inch and up to 4 or 6 inches or greater. It is conventional to form structures such as marine hulls from such steel plate by welding plates to each other and to a structural frame (such structures will be called hereinafter "plate structures"). The huge sizes of many plate structures very often place severe limitations upon the types of heat treatment which can be applied to the plates either before or after welding. For example, it is practically impossible to normalize, quench and temper any substantial portion of a hull of an ocean-going ship. Accordingly, it has been recognized that certain grades of alloy and/or carbon steels cannot be used successfully in plate applications since satisfactory welding of these steels requires pre-heating and/or the use of post-weld normalizing, quenching and tempering treatments. Among the many problems encountered with such alloy and/or carbon steels are cracking in the heat affected zone and welding-induced distortion.

Heat treatment problems are only some of the many difficulties which must be considered by an engineer designing a structure to be formed from plate. Weight and buoyancy considerations often require the designer to specify a steel of controlled high strength, i.e., a steel having a yield strength of about 140,000 pounds per square inch (p.s.i.) up to about 200,000 p.s.i. There are, of course, many steels which will exhibit yield strengths of such an order of magnitude. However, as indicated hereinbefore, the steel to be specified as plate must be weldable without heat affected zone (H.A.Z.) cracking under conditions encountered in the practical construction of large structures.

Another of the many considerations which is involved in the selection of a high strength plate steel is toughness of the plate. It is now well recognized that during rolling of plate, factors are brought into play which induce directional anomalies in mechanical characteristics in the final plate. As pointed out in the 8th edition of Metals Handbook, volume I, 1961 on pages 229 to 231, Charpy V-Notch (C.V.N.) specimens taken in a direction parallel to the direction of rolling often exhibit impact values substantially higher than the values exhibited by specimens taken in a direction transverse to the direction of rolling. In other words, longitudinal specimens taken parallel to the rolling direction show greater energy absorption than specimens taken in a transverse direction. Very often the difference between the energy absorption of transverse and longitudinal specimens can be of the order of 100% and higher based upon the transverse impact value. For example, the difference between the C.V.N. impact values in foot-pounds (ft.-lbs.) of transverse and longitudinal specimens of S.A.E. Steel No. 8617 taken at 0° F. is at least about 50 ft.-lbs. This difference is about 200% of the maximum C.V.N. impact value of 25 ft.-lbs., exhibited by transverse specimens of this steel at 0° F. with a hardness of 30 Rockwell C units (R<sub>c</sub>). Uniformly, in the 15 graphical representations set

## 2

forth on pages 230 and 231 of the Metals Handbook, the C.V.N. impact values of longitudinal specimens significantly exceed the C.V.N. impact values of transverse specimens. This directional phenomenon is particularly evident in rolled plate and sheet since the amount of work homogenization which can be induced in plate and sheet by cross rolling is limited by the length of the plate and/or sheet as opposed to the width of the available rolling mill. Thus, in the final stages of reduction of sheet and plate, it is often impossible to insert metal into a roll gap with the length of the sheet or plate parallel to the roll axes because the rolls are not wide enough. In contrast to rolled bar or rod (which are conventionally tested for toughness using longitudinal C.V.N. impact specimens) rolled plate and sheet almost inherently exhibit directional anomalies which are most evident in ascertaining toughness by the C.V.N. test.

The importance of the foregoing discussion to a designer of plate structures is clearly that the designer must design within toughness limits imposed by the lowest value of toughness criteria (usually impact values) exhibited by the materials available to him. It is also clear that the plate-structure designer must compare truly comparable impact values when deciding upon the relative merits of available material. Thus, for a designer to attempt to evaluate two plate steels solely by comparing C.V.N. impact values taken in one steel from transverse specimens and in the other steel from longitudinal specimens is a very unsound procedure unless the situation is such that the values exhibited by the transverse specimens of the one steel exceed the values exhibited by the longitudinal specimens of the other steel. In the latter situation it is perhaps safe to conclude that the steel from which transverse specimens were taken is at least as tough or tougher than the steel from which longitudinal specimens were taken.

In addition to the aforesaid factors of weldability, strength and toughness of the plate steel, a designer of plate structures must take into consideration the toughness of the weld-affected area in the assembled plate structure. It is known that many instances of brittle fracture of plate structures have originated in weld-affected areas of the structure. For example, on page 235 of the 1961 edition of the Metals Handbook, it is stated that the brittle fracture of a T2-type tanker occurring while the vessel was moored dockside, originated in a welding arc strike. On page 236 of the Metals Handbook, an example of the failure of a pressure vessel designed for petroleum refining is set forth. In this example, it is stated that during hydrostatic pressure testing, failure occurred in a knuckle plate at the base of a fillet weld. In view of the fact that in many instances, weld-affected areas of plate structures and cracks induced by welding are the originating points of brittle failures, it is necessary that a designer seriously consider the effect of welding upon the strength and toughness of the metal adjacent weld deposits. In this regard, it is not only necessary that commercially practical post-weld heat treatments give high strength efficiency in the weld-affected areas, but also such post-weld heat treatments must not detrimentally affect the toughness of the metal in the weld-affected areas to an extent that such toughness would fall below tolerable design limitations.

Keeping in mind all the foregoing difficulties and other problems, plate-structure designing and, in particular, specifying alloys for plate structures, is a very complex activity. As far as is known, the metallurgical art has never provided the designer with a wholly satisfactory commercial steel of controlled high strength suitable for use in plate structures adapted to be subjected in use to high pressures and violent impacts at temperatures

from above room temperature down to about  $-100^{\circ}$  F. and lower. Although many attempts were made to provide such a satisfactory, tough, controlled high strength plate steel, none, as far as we are aware, was entirely successful when carried into practice commercially on an industrial scale.

It has now been discovered that an alloy steel containing specially controlled and interrelated amounts of alloying elements is especially suited for use in the manufacture of plate structures having a high strength to weight ratio.

It is an object of the present invention to provide a novel steel.

Another object of the invention is to provide a novel maraged steel.

The invention also contemplates providing a novel process of heat treating said novel steel.

It is a further object of the invention to provide novel welded plate structures made from said novel steel.

The invention further contemplates providing a novel process of producing said novel plate structures.

Other objects and advantages will become apparent from the following description taken in conjunction with the accompanying drawing in which:

FIGURE 1 is a graphical representation of mechanical characteristics of a typical steel of the present invention as related to the aluminum content of the alloy; and

FIG. 2 is a graphical representation of the interrelation existing between yield strength and C.V.N. impact values as exhibited by alloys both within and without the present invention.

Broadly stated, the present invention contemplates novel maraging steel alloys consisting essentially, in percent by weight, of about 9.5% to about 13.5% nickel, about 2.5% to about 8% chromium, about 1.9% to about 4.2% molybdenum, about 0.05% to about 0.4% aluminum, up to about 0.30% titanium, and advantageously, about 0.1% to about 0.2% titanium, about 0.001% to about 0.03% carbon, up to not more than 0.25% manganese, up to about 0.30% silicon, up to about 0.01% boron, up to about 0.1% zirconium, with the balance being essentially iron in an amount of at least about 74%. The alloys can also contain impurities and incidental elements in small amounts which do not deleteriously affect the basic and novel characteristics of the alloy. Impurities such as sulfur, phosphorous, hydrogen, oxygen, nitrogen

than the aforesigned maximum amounts should be used and, in any event, no greater than 2% total of beryllium, vanadium, columbium, tantalum and tungsten should be present in alloys in accordance with the present invention.

More advantageous embodiments contemplated in accordance with the present invention include, with respect to alloy composition, alloys containing about 11% to about 12% nickel and/or about 3% to about 5% chromium and/or about 2.5% to about 3.5% molybdenum, and/or about 0.05% to about 0.15% aluminum and/or about 0.20% to about 0.30% aluminum. It is generally advantageous to limit the amount of chromium in the alloys of the invention to a maximum of about 5.5% in order to obtain the best combination of strength and toughness. The strength and toughness of the alloys of the present invention are also greatly dependent upon the aluminum content of the alloys. FIGURE 1 of the drawing shows that as the aluminum content of alloys in accordance with the invention (containing nominally 12% nickel, 5% chromium and 3% molybdenum) is increased from 0.1% to about 0.3%, the yield strength of the alloys increases sharply while the Charpy V-Notch impact values at  $70^{\circ}$  F. decrease only slightly. Above about 0.3% aluminum the impact values tend to decrease at an increasingly rapid rate to totally unacceptable levels. Consequently, it is important to specially maintain the amount of aluminum in the alloys of the invention below an ultimate maximum of 0.4% and, more advantageously, below about 0.35%. Each of the aforementioned more advantageous ranges of nickel, chromium, molybdenum and aluminum can be employed either singly or in combination with the ranges of alloy composition set forth hereinbefore. For reasons set forth in detail hereinafter, it is advantageous to interrelate the nickel and chromium contents within the aforementioned broader range and the more advantageous ranges so that the sum of the percentages of nickel and chromium in a given specific alloy is about 14% to about 19%. As high as about 0.50% silicon can be tolerated in alloys of the present invention provided that the aluminum copresent with amounts of silicon in excess of about 0.30% be no greater than about 0.30%.

The alloy ranges set forth in Table I are illustrative of the broadly stated and more advantageous alloy ranges of nickel, chromium, molybdenum, titanium and aluminum as set forth hereinbefore.

TABLE I

| Alloy Type | Percent C      | Percent Ni | Percent Cr | Percent Mo | Percent Al | Percent Ti | Percent Fe <sup>1</sup> |
|------------|----------------|------------|------------|------------|------------|------------|-------------------------|
| I-----     | 0.03 max-----  | 10-10.5    | 4.5-5      | 2-4        | 0.05-0.15  | 0.1-0.2    | Bal. E.                 |
| II-----    | 0.03 max-----  | 11.5-12.5  | 3-3.5      | 2.75-3.25  | 0.05-0.15  | 0.1-0.2    | Bal. E.                 |
| III-----   | 0.03 max-----  | 10-11      | 4-5        | 3-4        | 0.2-0.3    | 0.1-0.2    | Bal. E.                 |
| IV-----    | 0.03 max-----  | 11.5-12.5  | 3-5        | 2.5-3.5    | 0.2-0.3    | 0.1-0.2    | Bal. E.                 |
| V-----     | 0.025 max----- | 11.5-12.5  | 4.75-5.25  | 2.75-3.25  | 0.2-0.3    | 0.1-0.2    | Bal. E.                 |

<sup>1</sup> Bal. E. = balance essentially and includes the aforesigned small amounts of silicon, manganese, boron and zirconium together with small amounts of impurities and incidental elements.

and the like, should be kept at the lowest possible levels consistent with economical commercial production. Incidental elements such as cobalt and copper are not specifically beneficial in the alloys of the present invention and should be limited to those small amounts which are unavoidably introduced into the composition during commercial manufacture. Small amounts of elements such as beryllium, vanadium, columbium, tantalum and tungsten can be employed in the alloys of the present invention. These elements, when used singly, should be limited to the following maximum amounts: 0.2% beryllium, 1% vanadium, 0.4% columbium, 0.8% tantalum or 2% tungsten. When employed in combination, less

Alloys in accordance with the present invention have, at normal temperatures of usage, essentially a martensitic structure, that is, a structure resulting from a low temperature (below about  $700^{\circ}$  F.), substantially diffusionless transformation from austenite. During aging, as described in detail hereinafter, the alloys increase in hardness, for example, from about  $25 R_c$  to between about  $33 R_c$  and about  $43 R_c$ . This hardening response during aging distinguishes the alloys of the present invention from substantially all known prior art carbon steels (i.e., steels containing more than about 0.1% carbon) in that during tempering at temperatures akin to the aging tem-

peratures for the present alloys, prior art carbon steels exhibit a softening response.

Generally speaking, the alloys of the present invention are heat treated by a process which includes a first transformation to martensite after hot working, a solution anneal at a temperature in excess of about 1400° F., a second transformation to martensite following said solution anneal, and a final aging treatment in the vicinity of about 900° F. for a time in excess of about 1 hour and up to about 10 hours to harden and strengthen the alloy. As will be discussed hereinafter, the transformation to martensite can be accomplished by merely cooling the alloys to a temperature below about 150° F. The rate of cooling is not critical and drastic quenching operations are definitely not needed in order to obtain the advantageous mechanical characteristics of the alloys of the present invention.

Alloys according to the present invention are made by conventional high strength steel melting practice. For example, alloys of the present invention can be made by melting together relatively pure iron, nickel, chromium and molybdenum; decarburizing the resultant molten metal to produce a carbon level below about 0.03% by weight; deoxidizing the decarburized molten metal with silicon and manganese so as to limit residual silicon and especially residual manganese in the metal to within the aforementioned ranges for these elements; completing deoxidation by adding aluminum and titanium to provide residual amounts within the aforementioned ranges of aluminum and titanium; adding any desired boron and/or zirconium and casting the metal into ingots. In carrying out the manufacturing process, care must be taken to avoid introducing into the metal excessive amounts of sulfur, phosphorous, nitrogen, hydrogen and the like. Additions of small amounts of calcium which leave a residual of no more than about 0.02% in the metal can be beneficial in reducing sulfur to acceptable levels, e.g., about 0.01% maximum. Addition of malleableizing and deoxidizing amounts of rare earth elements (from the addition of misch metal), lithium, magnesium, uranium, etc., can be beneficial. Best results are obtained when premium grades of ingredients such as Armco iron, electrolytic nickel, electrolytic chromium and the like are employed in making alloys in accordance with the present invention. The alloys can be melted in high frequency induction furnaces advantageously under a blanket of inert gas such as argon. Alternatively, vacuum melting can be employed. Selected scrap can be used in the manufacture of alloys of the present invention provided proper basic electric furnace practice is employed and oxygen lancing is used to reduce carbon to levels below about 0.03%.

After the metal has been cast, the ingots are subjected to hot working operations at starting temperatures of about 2300° F., to mechanically homogenize the as-cast

therein. In the event sheet is desired, the cooled alloys can be worked further by hot-cold working and/or cold working to sheet thicknesses. After forming has been completed, the alloy is usually annealed at temperatures of about 1450° F. to about 1900° F. for about one to about four hours. The result of the annealing (or solution) treatment is to retransform any martensite to austenite, to place substantially all the alloying elements in solution in the matrix of the alloy and to remove the residual effects of hot and cold work.

Following annealing (or in special instances the finish of hot working) the alloy is cooled to room temperature or to a temperature at least below about 150° F. The rate of cooling after annealing is not critical but it is preferred to cool at a rate at least equal to the rate of air cooling. During cooling, the alloy structure changes from austenite (face-centered cubic) to martensite (body-centered cubic) by means of an essentially diffusionless process. The annealed martensitic alloy has a hardness of about 25 R<sub>c</sub>. Cold working, as mentioned hereinbefore, can be performed on the annealed martensitic alloy to the extent equivalent to about 90% reduction by rolling. Likewise, the annealed martensitic alloy of the present invention can be readily machined by sawing, drilling, turning, planing, milling and the like to final dimension. During subsequent aging, there is extremely little dimensional change.

After the annealed martensitic alloy has been formed or machined into the desired configuration, it is aged for about one to about ten hours at temperatures of about 800° F. to about 1000° F. A practical and recommended aging treatment is heating for about 3 hours at 900° F. During aging, samples of the annealed martensitic alloy increased in hardness from a level in the range of about 25 R<sub>c</sub> to about 32 R<sub>c</sub> in the annealed condition up to a level in the range of about 33 to 43 R<sub>c</sub> in the aged condition. Primarily depending upon composition, the yield strength of the aged alloys is of the order of about 140,000 p.s.i. to about 190,000 p.s.i. or even to about 200,000 p.s.i. The yield strength (Y.S.) level of aged samples of the alloy types disclosed in Table I are set forth in Table II:

TABLE II

| Alloy type: | Y.S., in p.s.i. |
|-------------|-----------------|
| I -----     | 145,000-155,000 |
| II -----    | 145,000-155,000 |
| III -----   | 165,000-175,000 |
| IV -----    | 165,000-175,000 |
| V -----     | 170,000-188,000 |

For the purpose of giving those skilled in the art a better understanding of the invention, examples of alloy compositions in accordance with the present invention are set forth in Table III:

TABLE III

| Alloy No. | Percent Ni | Percent Cr | Percent Mo | Percent Al | Percent Ti | Percent C | Percent Mn | Percent Fe <sup>1</sup> |
|-----------|------------|------------|------------|------------|------------|-----------|------------|-------------------------|
| 1-----    | 12.03      | 4.77       | 2.00       | 0.07       | 0.20       | 0.015     | <0.01      | Bal.                    |
| 2-----    | 12.04      | 2.95       | 3.00       | 0.12       | 0.18       | 0.011     | 0.03       | Bal.                    |
| 3-----    | 10.30      | 4.95       | 3.02       | 0.11       | 0.18       | 0.008     | 0.02       | Bal.                    |
| 4-----    | 12.09      | 3.25       | 2.07       | 0.23       | 0.20       | 0.008     | 0.04       | Bal.                    |
| 5-----    | 12.16      | 5.00       | 3.00       | 0.31       | 0.21       | 0.008     | <0.02      | Bal.                    |
| 6-----    | 10.26      | 4.87       | 4.03       | 0.31       | -----      | 0.009     | <0.02      | Bal.                    |
| 7-----    | 10.37      | 5.10       | 2.10       | 0.30       | -----      | 0.007     | <0.02      | Bal. <sup>2</sup>       |
| 8-----    | 9.67       | 4.90       | 1.95       | 0.21       | 0.10       | 0.025     | 0.08       | Bal.                    |
| 9-----    | 10.80      | 5.20       | 3.16       | 0.06       | 0.12       | 0.030     | 0.07       | Bal.                    |
| 10-----   | 10.05      | 4.73       | 4.18       | 0.07       | 0.12       | 0.027     | 0.07       | Bal.                    |

<sup>1</sup> Bal. means balance iron, inclusive of small amounts of silicon, boron, zirconium and/or calcium together with amounts of phosphorus below about 0.007% and sulfur below about 0.004%.

<sup>2</sup> Alloy No. 7 contains 0.48% silicon.

structure and to form hot rolled plate or other hot worked shapes. Finish hot working temperatures can be as low as about 1500° F. After hot working, the hot worked alloys are cooled to room temperature or at least below about 150° F. to induce a martensitic transformation

The alloys set forth in Table III, exhibit in the martensitic and age hardened condition the best combination of room temperature strength (as measured by yield strength) and room temperature toughness (as measured by C.V.N. values obtained with transverse specimens from

rolled plate). Additional examples of alloys in accordance with the present invention are set forth in Table IV:

TABLE IV

| Alloy No. | Percent Ni | Percent Cr | Percent Mo | Percent Al | Percent Ti | Percent C | Percent Mn | Percent Fe <sup>1</sup> |
|-----------|------------|------------|------------|------------|------------|-----------|------------|-------------------------|
| 11        | 10.40      | 5.15       | 2.16       | 0.40       | 0.19       | 0.008     | <0.01      | Bal.                    |
| 12        | 12.36      | 4.85       | 3.00       | 0.12       | 0.19       | 0.015     | 0.10       | Bal. <sup>2</sup>       |
| 13        | 11.17      | 3.85       | 2.55       | 0.19       | 0.19       | 0.010     | <0.02      | Bal.                    |
| 14        | 10.36      | 4.80       | 4.00       | 0.09       | 0.14       | 0.007     | <0.02      | Bal.                    |
| 15        | 12.05      | 2.94       | 2.93       | 0.05       | 0.13       | 0.032     | 0.06       | Bal.                    |
| 16        | 11.25      | 3.85       | 2.90       | 0.06       | 0.13       | 0.022     | 0.06       | Bal.                    |
| 17        | 10.20      | 4.72       | 2.95       | 0.05       | 0.12       | 0.031     | 0.06       | Bal.                    |
| 18        | 10.05      | 4.95       | 1.90       | 0.05       | 0.12       | 0.019     | 0.06       | Bal.                    |
| 19        | 10.28      | 2.85       | 3.00       | 0.32       | 0.21       | 0.006     | <0.02      | Bal.                    |

<sup>1</sup> Bal. means balance iron, inclusive of small amounts of silicon, boron, zirconium and/or calcium together with amounts of phosphorus below about 0.007% and sulfur below about 0.004%.

<sup>2</sup> Alloy No. 12 contains 0.31% silicon.

TABLE V

| Alloy No. | Hardness in Rc Units      |                          |
|-----------|---------------------------|--------------------------|
|           | Before Aging <sup>1</sup> | After Aging <sup>2</sup> |
| 1         | 25.0                      | 36.5                     |
| 2         | 25.5                      | 36.0                     |
| 3         | 25.5                      | 37.5                     |
| 4         | 25.5                      | 39.0                     |
| 5         | 27.5                      | 43.5                     |
| 6         | 30.5                      | 41.5                     |
| 7         | 28.0                      | 39.5                     |
| 8         | 27.5                      | 37.5                     |
| 9         | 31.5                      | 37.5                     |
| 10        | 32.0                      | 38.5                     |
| 11        | 28.5                      | 39.5                     |
| 12        | 26.5                      | 40.0                     |
| 13        | 26.5                      | 36.5                     |
| 14        | 28.0                      | 37.5                     |
| 15        | 26.0                      | 31.5                     |
| 16        | 28.5                      | 33.0                     |
| 17        | 31.0                      | 35.5                     |
| 18        | 27.5                      | 31.5                     |
| 19        | 24.5                      | 40.0                     |

<sup>1</sup> Annealed for 1 hour at 1500° F. followed by air cooling.

<sup>2</sup> Aged for 3 hours at 900° F. followed by air cooling.

The alloys as set forth in Tables III and IV were made by vacuum melting and/or by melting under an argon blanket as described hereinbefore. The carbon level of the molten metal was reduced by a carbon boil and initial deoxidation was accomplished by the use of silico-manganese. After all alloying ingredients were added, the metal was cast and hot worked as described hereinbefore to provide plate. The plates were then permitted to cool to room temperature to effect a first martensitic transformation therein. The alloys were then subjected to a solution treatment (annealing) at 1500° F. for 1 hour followed by cooling to room temperature to effect a second transformation to martensite. The alloys were then aged for 3 hours at 900° F. Hardnesses before and after aging are set forth in Table V:

The data set forth in Table V demonstrates that during aging at temperatures of about 800° F. to about 1000° F., the martensitic alloys of the present invention increase in hardness by up to about 15 Rockwell C units. After aging, the martensitic alloys of the present invention exhibit mechanical characteristics as set forth in Table VI.

TABLE VI

| Alloy No. | 0.2% Y.S., k.s.i. | U.T.S., <sup>1</sup> k.s.i. | E.I., <sup>2</sup> percent | R.A., <sup>3</sup> percent | C.V.N. Impact Strength (ft.-lbs.) <sup>4</sup> |          |          |
|-----------|-------------------|-----------------------------|----------------------------|----------------------------|------------------------------------------------|----------|----------|
|           |                   |                             |                            |                            | 70° F.                                         | -100° F. | -320° F. |
| 1         | 144.2             | 146.6                       | 16                         | 69                         | 111                                            | 86       | -----    |
| 2         | 145.1             | 149.3                       | 16                         | 73                         | 104                                            | 79       | -----    |
| 3         | 150.5             | 152.7                       | 17                         | 71                         | 95                                             | 69       | -----    |
| 4         | 163.6             | 169.1                       | 23                         | 71                         | 76                                             | 51       | -----    |
| 5         | 190.1             | 195.3                       | 15                         | 69                         | 45                                             | 32       | -----    |
| 6         | 181.9             | 184.7                       | 15                         | 69                         | 50                                             | 35       | -----    |
| 7         | 163.5             | 165.9                       | 17                         | 66                         | 70                                             | 31       | -----    |
| 8         | 166.3             | 166.3                       | 16                         | 70                         | 87                                             | 51       | -----    |
| 9         | 173.9             | 173.9                       | 17                         | 68                         | 62                                             | 44       | 28       |
| 10        | 171.9             | 171.9                       | 20                         | 69                         | 57                                             | 40       | 16       |
| 11        | 168.8             | 170.8                       | 15                         | 65                         | 49                                             | 35       | -----    |
| 12        | 165.7             | 170.5                       | 18                         | 65                         | 60                                             | 43       | -----    |
| 13        | 147.5             | 149.9                       | 18                         | 70                         | 88                                             | 67       | -----    |
| 14        | 154.6             | 157.4                       | 17                         | 68                         | 51                                             | 43       | -----    |
| 15        | 149.9             | 149.9                       | 22                         | 73                         | 78                                             | 58       | 40       |
| 16        | 155.0             | 155.0                       | 19                         | 72                         | 68                                             | 52       | 31       |
| 17        | 158.9             | 159.0                       | 18                         | 70                         | 56                                             | 36       | 23       |
| 18        | 147.1             | 147.1                       | 22                         | 73                         | 88                                             | 62       | 41       |
| 19        | 166.7             | 170.7                       | 15                         | 54                         | 53                                             | -----    | -----    |

<sup>1</sup> U.T.S., is ultimate tensile strength measured in thousands of pounds per square inch (k.s.i.).

<sup>2</sup> E.I. is elongation expressed in percent based upon a gage length of 4 times the test bar diameter.

<sup>3</sup> R.A. is reduction in area expressed in percent and based upon the cross-sectional area of the gage length of the test bar.

<sup>4</sup> Values obtained from plate samples. Impact specimens were cut in a direction transverse the direction of rolling.

In addition to the mechanical characteristics set forth in Table VI, which are representative of the mechanical characteristics of aged martensitic alloys in accordance with the present invention, alloys of the present invention also exhibit excellent notch tensile strengths of the order of 1.5 (or greater) times the ultimate tensile strength. It is also characteristic of alloys of the present invention that the ratios of yield strength to ultimate tensile strength are in excess of 0.9 and usually in excess of 0.95.

In the as-annealed condition, i.e., after solution treatment at 1500° F. for 1 hour, followed by air cooling, alloys in accordance with the present invention also exhibit an excellent combination of characteristics. The data set forth in Table VIA illustrates this with respect to alloys containing, in addition to the indicated aluminum percentages, nominally about 12% nickel, 5% chromium, 3% molybdenum, about 0.01% carbon, with the balance being essentially iron.

TABLE VIA

| Percent Al | Y.S., k.s.i. | U.T.S., k.s.i. | El., percent | R.A., percent | C.V.N. <sup>1</sup> (ft.-lbs.) |
|------------|--------------|----------------|--------------|---------------|--------------------------------|
| 0.17-----  | 106          | 140.2          | 18           | 74.5          | 102                            |
| 0.29-----  | 102.5        | 143.2          | 16           | 76.2          | 97                             |

<sup>1</sup> At room temperature.

As indicated hereinbefore, weld-affected areas of aged martensitic alloys of the present invention can be restored in properties by a simple postweld heat treatment at about 900° F. Such a heat treatment can be applied to a large welded plate structure by means, for example, of strip heaters, electrical resistance heating, induction heating, torch heating, etc. Macro and micro examinations of the weld-affected areas of welded plate samples disclosed only sound metal with no discernible cracks. During welding, heat affected zones of the metal of the welded samples softened somewhat. Subsequent maraging resulted in complete restoration to the hardness of the plate body. In cruciform welding tests embodying a high degree of restraint, no cracking was discernible in heat affected zones of 1 inch plate samples in accordance with the present invention.

To achieve the objects of the present invention, it is vitally important that the chemical composition of the alloys of the present invention be maintained within the limits of the ranges set forth hereinbefore. The nickel

Both chromium and molybdenum within the ranges of about 2.5% to 5.5% and about 2% to about 4%, respectively, are advantageous because with amounts of these elements lower than those specified, alloys of much lower strength are attained. Increasing the amounts of molybdenum above those specified as a maximum results in drastically lowering the toughness of the alloys and lowering strength. An excessive amount of chromium in the alloy tends to lower strength. Amounts of chromium in excess of about 5.5% and up to about 8% can be advantageous from a corrosion standpoint. Amounts of manganese above about 0.25%, which are normally considered as beneficial in good alloy steel manufacturing practice, are detrimental to the toughness of the alloys of the present invention and, accordingly, the maximum manganese permitted in the alloys of the present invention is about 0.25%. It is essential that in the presently disclosed alloys the carbon be kept at a maximum of about 0.03%, i.e., less than 0.033%. Amounts of carbon even slightly in excess of 0.033% have a deleterious effect on toughness of the alloys. Raising carbon in the alloys of the present invention to very (comparatively speaking) high levels of 0.1% or more, results in the production of alloys akin to known carbon steels, said alloys having the defects and deficiencies of carbon steels as discussed in detail hereinbefore. The maximum specified carbon content is also highly critical in that the deleterious effects of amounts in excess of about 0.03% in the alloys of the invention cannot be remedied by the use of carbide formers such as titanium. Like carbon, metal carbides such as titanium carbide, drastically reduce the toughness of alloys which otherwise would be within the ambit of the present invention. Amounts of aluminum up to about 0.3% or 0.4% assist in strengthening the alloys of the present invention as shown in FIGURE 1 of the drawing. Titanium in amounts up to about 0.3%, e.g., about 0.1% to about 0.2%, in combination with less than about 0.03% carbon is advantageous in that it tends to minimize the deleterious effects of small amounts of sulfur which may inadvertently be present in the alloys.

The critical nature of composition limits discussed hereinbefore is exemplified by reference to Tables VII and VIII. Compositions of alloys (designated by letters) outside the present invention are set forth in Table IX together with compositions of alloys (designated by numbers) within the present invention to provide a comparison.

TABLE VII

| Alloy   | Percent Ni | Percent Cr | Percent Mo | Percent Al | Percent Ti | Percent C | Percent Mn | Percent Fe        |
|---------|------------|------------|------------|------------|------------|-----------|------------|-------------------|
| A-----  | 12.10      | -----      | 3.01       | 0.06       | 0.14       | 0.021     | 0.06       | Bal. <sup>1</sup> |
| 9-----  | 10.80      | 5.20       | 3.16       | 0.06       | 0.12       | 0.030     | 0.07       | Bal. <sup>1</sup> |
| B-----  | 11.95      | 3.43       | 1.01       | 0.24       | 0.10       | 0.021     | 0.06       | Bal. <sup>1</sup> |
| C-----  | 10.25      | 4.55       | 5.20       | 0.07       | 0.11       | 0.028     | 0.07       | Bal. <sup>1</sup> |
| 4-----  | 12.09      | 3.25       | 2.07       | 0.23       | 0.20       | 0.008     | 0.04       | Bal. <sup>1</sup> |
| D-----  | 9.80       | 2.75       | 2.88       | 0.06       | 0.12       | 0.04      | -----      | Bal. <sup>1</sup> |
| E-----  | 11.90      | 3.18       | 3.30       | 0.06       | 0.11       | 0.05      | -----      | Bal. <sup>1</sup> |
| F-----  | 11.50      | 4.75       | 2.00       | 0.26       | 0.10       | 0.06      | 0.07       | Bal. <sup>1</sup> |
| G-----  | 10.00      | 4.80       | 2.00       | 0.25       | 0.20       | 0.06      | 0.07       | Bal. <sup>1</sup> |
| H-----  | 12.6       | 5.4        | 2.9        | 0.22       | 0.14       | 0.023     | 0.29       | Bal. <sup>1</sup> |
| I-----  | 12.5       | 5.5        | 3.0        | 0.11       | 0.13       | 0.024     | 0.29       | Bal. <sup>1</sup> |
| J-----  | 12.4       | 5.5        | 3.0        | 0.14       | 0.14       | 0.024     | 0.42       | Bal. <sup>1</sup> |
| 20----- | 12.08      | 4.87       | 2.97       | 0.25       | 0.15       | 0.099     | 0.10       | Bal. <sup>1</sup> |
| 21----- | 12.26      | 4.98       | 2.97       | 0.23       | 0.14       | 0.015     | 0.21       | Bal. <sup>1</sup> |
| 5-----  | 12.16      | 5.00       | 3.00       | 0.31       | 0.21       | 0.008     | <0.02      | Bal. <sup>1</sup> |
| K-----  | 10.4       | 6.4        | 0.76       | 0.022      | 0.18       | 0.122     | 0.44       | Bal. <sup>2</sup> |
| L-----  | 10.3       | 6.5        | 0.77       | 0.024      | 0.16       | 0.113     | 0.38       | Bal. <sup>2</sup> |

<sup>1</sup> Bal. means balance iron, inclusive of small amounts of silicon, boron, zirconium and/or calcium, together with amounts of phosphorus below about 0.007% and sulfur below about 0.004%.

<sup>2</sup> Also contain about 0.45% copper.

content must be maintained within the range of about 9.5% to about 13.5% because lower amounts of nickel, especially in combination with amounts of chromium below about 3%, lead to decreased strength and to decreased low temperature toughness characteristics. Amounts of nickel higher than about 13.5% are uneconomical and, in association with high chromium, lead to lower strength.

All of the alloys in Table VII were made, worked and heat treated in accordance with the procedure disclosed hereinbefore as to alloys of Tables III and IV. Duplicate samples of alloys K and L after melting, casting and working to plate in the usual manner were first normalized at 1625° F., second normalized at 1450° F. and tempered

at 1050° F. Mechanical characteristics of the alloys of Table VII are set forth in Table VIII.

loys D, E, F, G, K and L of Table VII. As set forth in Table VIII, none of these alloys exhibit a room tempera-

TABLE VIII

| Alloy          | 0.2% Y.S.,<br>k.s.i. | U.T.S.,<br>k.s.i. | El.,<br>percent | R.A.,<br>percent | C.V.N. Impact Strength<br>(ft.-lbs.) <sup>1</sup> |          |          |
|----------------|----------------------|-------------------|-----------------|------------------|---------------------------------------------------|----------|----------|
|                |                      |                   |                 |                  | 70° F.                                            | -100° F. | -320° F. |
| A              | 129.1                | 129.5             | 22              | 75               | 89.5                                              | 63.5     | 38.0     |
| 9              | 173.9                | 173.9             | 17              | 68               | 62                                                | 44       | 28       |
| B              | 136.5                | 136.7             | 19              | 71               | 46                                                | 40       | —        |
| C              | 185.3                | 185.3             | 17              | 64               | 25.5                                              | 27       | 11.5     |
| 4              | 163.6                | 169.1             | 23              | 71               | 76                                                | 51       | —        |
| D              | 162.9                | 162.9             | 17              | 66               | 34                                                | 22.5     | 18       |
| E              | 169.8                | 169.8             | 18              | 65               | 29                                                | 25       | 16       |
| F              | 199.7                | 203.6             | 14              | 59               | 25                                                | 19.5     | 8        |
| G              | 170.5                | 172.1             | 15              | 65               | 30                                                | —        | —        |
| H              | 182.2                | 183.6             | 15              | 62               | 31.5                                              | 25.5     | 5.5      |
| I              | 172.7                | 177.4             | 15              | 63               | 34.5                                              | 27       | 6        |
| J              | 180.6                | 184.4             | 15              | 61               | 32.5                                              | 27       | 5.5      |
| 20             | 178.6                | 183.2             | 16              | 62.5             | 51                                                | 43       | —        |
| 21             | 173.3                | 177.6             | 15              | 66               | 57                                                | 41.5     | —        |
| 5              | 190.1                | 195.3             | 15              | 69               | 45                                                | 32       | —        |
| K <sup>2</sup> | 123.5                | 146.0             | 20              | 64               | 26                                                | 24.5     | 20       |
| L <sup>2</sup> | 143.9                | 147.8             | 21              | 64               | 33                                                | 32       | —        |
| K              | 176.9                | 181.9             | 16              | 60               | 16                                                | 15.5     | 11       |
| L              | 172.3                | 174.5             | 17              | 63               | 26.5                                              | 21       | 13       |

<sup>1</sup> Values obtained from plate samples—Impact specimens were cut in a direction transverse to the direction of rolling.

<sup>2</sup> Heat treated by double normalizing followed by tempering at 1,050° F.

The data set forth in Table VIII is to be considered in conjunction with FIG. 2 of the drawing. FIG. 2 of the drawing shows the interrelation between 0.2% yield strength and room temperature (70° F.) Charpy V-Notch impact strengths of alloys set forth in the present specification. It is known in general for steels that there is an inverse relationship between strength and toughness. Thus, for any given steel as the strength is increased, the toughness decreases. For alloys in accordance with the present invention containing alloying elements within the ranges set forth in Table IX, this inverse relationship is generally representable by approximately the curve DE as shown in FIG. 2.

TABLE IX

| Element    | Percent<br>By Weight | Element   | Percent By Weight    |
|------------|----------------------|-----------|----------------------|
| Nickel     | 9.5 - 13.5           | Titanium  | About 0.3 max.       |
| Chromium   | 2.5 - 5.5            | Carbon    | About 0.03 max.      |
| Molybdenum | 1.9 - 4.2            | Manganese | 0.15 max.            |
| Aluminum   | 0.05-0.40            | Silicon   | 0.30 max.            |
|            |                      | Iron      | Balance Essentially. |

Further, with respect to alloys of the present invention having compositions falling (except for manganese and silicon) within the ranges set forth in Table IX, the curves AB and BC effectively define the minimum strength and toughness limits obtainable. Such alloys can be represented by a point lying above and to the right of curves AB and BC when heat treated in accordance with the presently disclosed process to 0.2% yield strengths of about 140 k.s.i. to about 200 k.s.i. As a general approximation, such alloys are characterized by 0.2% yield strengths and room temperature C.V.N. impact strengths such that both of the following quasi-mathematical criteria are satisfied:

$$Y.S. + 4.1(C.V.N.) = > 350$$

$$Y.S. + 0.20(C.V.N.) = > 163$$

Alloys as set forth in Table IX always exhibit a room temperature C.V.N. impact value in excess of about 40 foot-pounds. The effect of raising carbon even slightly above about 0.03% is dramatically demonstrated by al-

ture C.V.N. impact strength as high as 40 foot-pounds. The yield strengths and impact strengths of alloys D, E, F, G, K and L have been plotted on FIG. 2 of the drawing (as circles) and can be compared to the yield strengths and impact strengths of the alloys of the present invention plotted (as X's) on the same figure. Tables VII and VIII also show that when chromium is deleted from the alloys of the present invention the strength is low; that when molybdenum is below about 1.9% the strength and toughness is low; that when molybdenum exceeds about 4.2% the toughness is low; and that when manganese exceeds about 0.25% (alloys H, I and J) the toughness of the alloys is low.

When the chemistry of the alloys of the present invention is controlled within the more advantageous limits set forth hereinbefore and welds are made with suitable and compatible fillers, highly advantageous weld joints can be produced. Tests have shown that in tungsten-inert-gas weld joints of  $\frac{1}{2}$  inch plate samples of alloys in accordance with the present invention, combinations of characteristics as set forth in Table X can be obtained.

TABLE X

|                              | Room temperature<br>C.V.N. values,<br>ft.-lbs. |    |
|------------------------------|------------------------------------------------|----|
| 0.2% yield strength, k.s.i.: |                                                |    |
| 155                          | —                                              | 70 |
| 165                          | —                                              | 60 |
| 175                          | —                                              | 50 |

The ranges of alloying elements in accordance with the present invention as set forth hereinbefore include certain interrelationships among alloying elements. One of the essential concepts of the present invention is that in alloys in accordance with the invention, the total nickel plus chromium content must be between about 13.5% and about 19%. When nickel and chromium are co-present in the alloys of the present invention in the amounts set forth hereinbefore, these elements appear to interact during maraging (i.e., aging in the martensitic condition after martensitic transformation), to harden and strengthen the alloy. This interaction during maraging is most pronounced when the nickel content is about 11% to about 12%, the chromium content is about 3% to

about 5% and the total of the nickel plus chromium is about 14% to about 16%. It is essential that at least 0.05% aluminum be present in the alloys of the present invention. As shown in FIGURE 1 of the drawing, aluminum in amounts between about 0.1% and 0.3% contributes greatly to the strength of the alloys and permits this strength to be attained without great sacrifice of toughness.

The present invention is particularly applicable to the provision of plate for high strength, welded structures. Examples of such structures are ships' hulls, pressure vessels for chemical reactors and high pressure equipment, rotors for electrical generators, etc. The alloys of the present invention can, of course, be provided in forms other than plate, for example, sheet, bar, rod, wire, strip, tube and the like. These forms can be produced by hot working, e.g., forging, rolling, extrusion and the like, cold working, e.g., rolling, drawing, pressing, etc., hot-cold working, machining including turning, drilling, milling and the like and, in general, by any conventional shaping or cutting operation used in ferrous metal technology. While not necessary in the usual instance, the alloys of the present invention can be formed by any of the relatively new high-energy processes, including high-energy impact processes and explosive forming. The alloys of the present invention can also be provided with a hard surface by conventional low temperature nitriding.

It is to be observed that the present invention provides a novel maraging steel having in the age hardened condition highly useful levels of strength in excess of about 140 k.s.i. yield strength coupled with high levels of toughness indicated by C.V.N. impact values in transverse plate samples at room temperatures in excess of about 70 ft.-lbs. at yield strengths up to about 150 k.s.i. and in excess of about 50 ft.-lbs. at yield strengths up to about 170 k.s.i. or higher. This advantageous combination of strength and toughness is highly useful since it can be readily attained in welded plate structures. The alloys also exhibit advantageous combinations of mechanical characteristics at cryogenic temperatures. For example, in general the alloys of the present invention exhibit C.V.N. impact values of the order of 30 to 60 ft.-lbs. at -100° F. and C.V.N. impact values of the order of 20 to 40 ft.-lbs. at -320° F. Other metals such as alloy carbon steels cannot, under commercial conditions, attain the required strength and toughness combination in welded plate structures without resorting to uneconomical and/or technically impractical pre- and/or postweld heat treatments.

Although the present invention has been described in conjunction with preferred embodiments, it is to be understood that modifications and variations may be resorted to without departing from the spirit and scope of the invention, as those skilled in the art will readily understand. Such modifications and variations are considered to be within the purview and scope of the invention and appended claims.

We claim:

1. A maraging steel for use at 0.2% yield strengths in excess of about 140,000 pounds per square inch in thick sections in plate structures consisting essentially, in weight percent, of about 9.5% to about 13.5% nickel, about 2.5% to about 8% chromium, said nickel and said chromium being interrelated so that the sum thereof is about 13.5% to 19%, about 1.9% to about 4.2% molybdenum, about 0.05% to about 0.40% aluminum, up to about 0.3% titanium, about 0.001% to about 0.03% carbon, up to about 0.25% manganese, up to about 0.50% silicon with the silicon content not exceeding about 0.3% when the aluminum exceeds about 0.3%, up to about 0.01% boron, up to about 0.1% zirconium, up to about 2% total of metal from the group consisting of beryllium, vanadium, columbium, tantalum and tungsten, said elements in said group being present individually in

amounts of 0% to 0.2% beryllium, 0% to 1% vanadium, 0% to 0.4% columbium, 0% to 0.8% tantalum and 0% to 2% tungsten, the balance of the steel being essentially iron in an amount of at least about 74%.

5 2. A plate structure made of the maraging steel of claim 1.

3. The steel composition as set forth in claim 1 in which the silicon content does not exceed about 0.3%.

4. A steel as in claim 1 heat treated by subjecting said 10 steel to a first martensitic transformation, annealing said steel to convert the thus-formed martensite to austenite, cooling the annealed steel to effect a second transformation to martensite and thereafter aging the thus-treated martensitic steel at about 800° F. to about 1000° F. to increase the 0.2% yield strength thereof to at least about 15 140,000 pounds per square inch.

5. A maraging steel for use at 0.2% yield strengths in excess of about 140,000 pounds per square inch in thick 20 sections in plate structures consisting essentially, in weight percent, of about 9.5% to about 13.5% nickel, about 2.5% to 5.5% chromium, said nickel and said chromium being interrelated so that the sum thereof is about 13.5% to 17%, about 1.9% to about 4.2% molybdenum, about 0.05% to about 0.40% aluminum, up to about 0.3% titanium, about 0.001% to about 0.03% carbon, up to about 0.25% manganese, up to about 0.50% silicon with the silicon content not exceeding about 0.3% when the aluminum exceeds about 0.3%, up to about 0.01% boron, up to about 0.1% zirconium, up to about 20 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 977

## 15

10. A maraging steel consisting essentially, in weight percent, of about 10% to about 12.5% nickel, about 3% to about 5.5% chromium, the total of said nickel and said chromium being at least about 14%, about 2% to about 4% molybdenum, about 0.05% to about 0.3% aluminum, about 0.1% to about 0.2% titanium, up to about 0.03% carbon, up to about 0.25% manganese, up to about 0.3% silicon, with the balance being essentially iron.

11. A plate structure made of the maraging steel of claim 10.

12. A maraging steel as in claim 10 containing about 2.5% to about 3.5% molybdenum.

## 16

## References Cited by the Examiner

## UNITED STATES PATENTS

|             |         |                     |           |
|-------------|---------|---------------------|-----------|
| 2,999,039   | 9/1961  | Lula et al. -----   | 148—37    |
| 3,093,519   | 6/1963  | Decker et al. ----- | 148—142 X |
| 5 3,123,506 | 3/1964  | Tanczyn -----       | 148—31    |
| 3,151,978   | 10/1964 | Perry et al. -----  | 148—37    |
| 3,164,497   | 1/1965  | Matsuda -----       | 148—142   |

HYLAND BIZOT, Primary Examiner.

10 DAVID L. RECK, Examiner.

C. N. LOVELL, Assistant Examiner.